

May 13, 1930.

M. U. SCHOOP

1,758,473

COATING ARTICLES PARTICULARLY WITH METALS

Filed June 26, 1925.

3 Sheets-Sheet 1



Inventor:

May U. Schoop:

By *Henry Orth* atty.

May 13, 1930.

M. U. SCHOOP.

1,758,473

COATING ARTICLES PARTICULARLY WITH METALS

Filed June 26, 1925

3 Sheets-Sheet 2



Inventor:

May U. Schoop.

By  Atto.

May 13, 1930.

M. U. SCHOOP

1,758,473

COATING ARTICLES PARTICULARLY WITH METALS

Filed June 26, 1925

3 Sheets-Sheet 3



Fig. 7



Fig. 8

Inventor:

Max U. Schoop,  
By *Henry Smith*

Atty.

## UNITED STATES PATENT OFFICE

MAX ULRICH SCHOOP, OF HOENGG, SWITZERLAND

COATING ARTICLES, PARTICULARLY WITH METALS

Application filed June 28, 1925, Serial No. 39,785, and in Switzerland June 30, 1924.

The present invention relates to improvements in a method and a device for coating articles and particularly for producing metallic coatings.

With the present method the coating material is no longer used in the form of a wire as with the known metal spraying apparatus designed as pistol, but in the form of metallic powder or metallic bronzes which are in 10 a convenient manner melted to the surface of the article to be coated by means of a reducing melting flame. Thereby exceedingly fine and strongly adhering layers are obtained which cannot be distinguished from 15 galvanic coatings and which show a homogeneous metallic continuity.

The so-called metallic bronze is the most suitable coating material. The present invention has little in common with the known 20 method of projecting the molten particles of a wire towards the surface and the apparatus for carrying into effect the present method has no longer any resemblance with the spraying pistol; any burner used for 25 autogenous welding may be utilized.

The characterizing features of the new layers are thus essentially different from those obtained by the method utilizing the pistol.

30 Constructional examples of the subject matter of the present invention are illustrated on the accompanying drawings in which:

Fig. 1 shows a welding burner of the injector type having a controlling screw for the acetylene and oxygen supply.

Fig. 2 shows the burner according to Fig. 1 provided with a nozzle head for producing the coatings.

40 Fig. 3 shows the nozzle head.

Fig. 4 is a detail of nozzle head, Fig. 3.

Fig. 5 shows an apparatus partly in section.

45 Fig. 6 is a longitudinal section of a nozzle head which may be used on the apparatus Fig. 5.

Fig. 7 shows another form of apparatus, and

50 Fig. 8 illustrates an apparatus in which

the impelling vapor pressure is produced from the reducing medium used.

In Fig. 3 the supply for the constituent parts of combustion gas, for instance acetylene-oxygen is designated by 1; 2 is the channel along which the metallic bronze is fed, 3 is the supply conduit for the pressure medium, for instance compressed air, which has to accomplish two tasks: (a) to increase the speed of flow of the metallic particles, (b) to 60 reduce the temperature of the flame which is too high in most cases. The inner mouth piece 4 of the nozzle (Fig. 4) is preferably provided with helical grooves 5 in order to impart a swirling or rotating motion to the 65 mixture of air and metal at the exit. Thereby by an intimate contact with and distribution of the particles in the reducing zone of the flame is ensured.

The oxygen-acetylene flame has strongly 70 reducing properties and this is advantageous as the products obtainable in the trade are mostly oxidized. When the flame cone as well as the feed of the metal are properly adjusted it is, possible for instance to produce nice compact coatings of the normal typical salmon red of sound copper from dark coloured strongly oxidized copper powder.

The novel method of applying a coating by 75 melting or welding is technically and economically superior to the known spraying process as may be seen with reference to Figs. 1-4. The apparatus does not require any movable, delicate parts, no turbine for 80 feeding the material, no ball bearings and does not have the characteristics of a sensitive precision instrument. The coatings are 85 bright and, as has been mentioned above, of an extraordinary density and smoothness; 90 they do not require any further treatments (such as grinding or polishing), which treatments are in most cases as expensive as the 95 production of the coating. The cleaning by means of the sand blast apparatus is no longer required, the surfaces to be coated have only to be freed from grease. The metallic particles are in a molten state when they 100 reach the surface to be coated, the latter is well heated by the oxygen-acetylene flame

and the result is a so to speak welded-on, brilliant and dense metallic coating.

Numerous tests and observations have shown that the method is improved and simplified if the metallic bronze is introduced into the channel by means of the inflammable gas. Each single metallic particle is then forced to pass the reducing zone of the flame and to melt thereby. The possibility of insufficiently heated particles rebounding from the surface to be coated is then totally excluded, i. e. all of the metal of the powder is melted, a result of extraordinary technical, hygienic and economic importance.

In order to impart a greater speed of flow to the molten particles extruding together with the inflammable gas and to reduce at the same time the temperature of the flame cone which is too high in most cases, compressed air is fed at the mouth of the nozzle in a convenient manner for instance concentrically or through a slot, the quantity and the pressure of the compressed air being the greater, the lower the fusing point of the coating metal is. This knack ensures that no metallic dust or vapour are generated, which molests the operators. The quantity of air supplied to and surrounding the flame controls its temperature, and the operator soon acquires the facility of adjusting this quantity to the various conditions of the temperature at the time of use.

These conditions are dependent upon the pressure of the gas or vapor propelling the metal powder, the inflammability of this vapor, the melting point of the metal, the size of powder particles, their condition of oxidation, and other conditions.

If the quantity of air is too great this will be indicated by a rebound of metal dust from the article being coated, if too small, either by too fluid metal deposit or by vaporization of the metal powder. With metals having a low fusing point, such as for example tin or lead, mixtures of gases may be employed which give low temperatures (i. e. mixtures of illuminating gas and air or of hydrogen and air).

Figs. 5 and 6 of the drawing serve to illustrate an apparatus by means of which a rudimentary experiment can be carried out showing the essence of the invention. The mixture of gas fed to an ordinary acetylene welding burner is led into a bottle 9 (Fig. 5), the contents of which, consisting for instance of copper powder, is whirled at  $\omega$  by the gas leaving the pipe 10 and is carried away through the pipe 11 to the burner 12; the two arrows at the mouth of the burner indicate the compressed air which is fed concentrically to the burner.

Fig. 6 shows in an axial section the mouth piece 12 of the burner, 12<sup>a</sup> denoting the channel through which flows the gaseous mixture containing the metallic powder in suspen-

sion and 12<sup>b</sup> is the conduit for supplying compressed air.

The experiments may also be carried out by feeding pulverized coating material from a suitable container by gravity and in a controllable manner into the gas channel, the closed container being subjected to pressure for obtaining an equalization of pressure. An apparatus of this type is illustrated in a diagrammatic manner in Fig. 7 in which 9 denotes the container having a conical bottom 13. A vertical feed screw 14 is provided which controls the discharge of the pulverized material at the bottom of the container 9. The combustible mixture flows through the conduit 15 which ends in a nozzle 16 and creates a suction action on the material discharged into the annular space 17 surrounding the nozzle 16. The pipe leads the coating material suspended in the stream of combustible gas to the burner. The feed screw 14 may be rotated by means of the bevel gear 19, 20 by a horizontal shaft 21 driven by any means for instance by a pulley 22.

Another manner of feeding the pulverized metallic particles is illustrated in Fig. 8. The material to be coated is mixed with an easily evaporable liquid for instance benzol, petrol, amyacetate and the like in a closed container 23 which is heated by a burner indicated at 24. A pipe 25 extends from above to near the lower end of the receptacle 23 and the boiling mixture raises under the influence of the steam pressure and conveys thus the pulverized material over any length through the pipe 26. The latter ends in a nozzle 27 surrounded by the annular nozzle 28 to which the combustible gas or oxygen is supplied through the pipe 29. Near the end of the pipe 26 a further burner 30 may be arranged which completely evaporates the liquid in which the coating material is suspended so that a mixture of vapour and pulverized material is discharged at the nozzle 27. This device of feeding the pulverized coating material ensures a perfectly uniform supply of the latter. Attention may be drawn to the fact that the velocity of the flowing combustible gas must exceed the flame velocity of the explosive mixture. Obviously the same ultimate result is obtained if instead of the finished explosive mixture oxygen is utilized for transporting the metallic powder and the two gases are caused to mix only at the mixing cock or the burner respectively.

It will be recognized how extremely simple and handy the whole metallizer apparatus has become especially if compared with the old metallizer pistol working with wire.

I claim:

A process of producing coatings which comprises mixing a metal powder with liquid combustible in a closed container, heating the mixture to produce a vapor pressure on

the surface of the mixture to expel the mixture, heating the mixture after expulsion to vaporize the liquid content of the mixture and increase the velocity of the now vapor and metallic particle mixture, and burning the resultant mixture in a jet.

In testimony whereof, I have signed my name to this specification.

DR. MAX ULRICH SCHOOP.

10

15

20

25

30

35

40

45

50

55

60